# EUROPEAN PATENT APPLICATION

(11) **EP 1 743 775 A1**
(43) Date of publication of application: **17.01.2007**
(21) Application number: 05106431.9
(22) Date of filing: 13.07.2005
(51) Int. Cl.: B41M 5/00, B41M 1/06, D21H 19/36, D21H 19/82, D21H 19/84

(54) **Coated paper for sheet fed offset printing**

(71) Applicant: SAPPI Netherlands Services B.V., 6211 AA Maastricht (NL)
(72) Inventor: Haenen, JP. G. H. F, 6245 Eysden (NL); Resch, P.K, 8071 Vasoldsberg (AT); Scholte H.B, 6132 GJ Sittard (NL)
(74) Representative: Bremi, Tobias Hans

(57) **Abstract**

SUMMARY

The specification pertains to a single or multiple coated printing sheet in particular but not exclusively for sheet-fed offset printing with an image receptive coating layer on a paper substrate. The printing sheet has the property that it can be printed in an offset printing process without spraying a fine powder, usually called offset powder or dust powder, on the sheet as it comes off the press to prevent the ink from transferring to the back side of the next sheet. Also irradiative (UV or IR) or heat drying on the sheet fed press is not necessary and/or the use of overprint varnish is not required. In addition to that, unexpectedly short converting times and times until reprinting is possible can be achieved. Furthermore methods for making such a printing sheet and uses of such a printing sheet are disclosed.

## Description

### TECHNICAL FIELD

The present invention pertains to a single or multiple coated printing sheet in particular, but not exclusively, for sheet-fed offset printing, with an image receptive coating layer on a paper substrate. The invention furthermore pertains to methods for making such a coated printing sheet and to uses of such coated printing sheets.

### BACKGROUND OF THE INVENTION

In the field of sheet fed offset printing it is desirable to be able to further process of freshly printed sheet as quickly as possible, while at the same time still allowing the printing inks to settle in and on the surface of the paper in a way such that the desired print gloss and the desired resolution can be achieved. Relevant in this context are on the one hand the physical ink drying process, which is connected with the actual absorption of the ink vehicles into an image receptive coating, e.g. by means of pores provided therein, and with the evaporation of solvents. The physical ink drying process may for example be supported by additional heating on the sheet fed press such that the evaporation of the solvent takes place efficiently or by IR or UV-irradiation. On the other hand there is the so-called chemical drying of the ink, which is connected with solidification of the ink in the surface and on the surface of the ink receptive layer, which for example takes place due to a cross-linking of cross linkable constituents of the inks. This chemical drying process can on the one hand also be assisted by heating, it may however also be sped up by adding specific chemicals to the inks which support the cross-linking process.

Nowadays typically converting times and times until reprinting as possible is in the range of several hours, which is a severe disadvantage of the present ink and/or paper technology, since it slows down the printing processes and makes intermediate storage necessary.

### SUMMARY OF THE INVENTION

The objective problem underlying the present invention is therefore to provide an improved printing sheet, single coated or multiple coated, in particular for sheet fed offset printing. The printing sheet shall be provided with an image receptive coating layer on a paper substrate, and it shall allow to simplify the printing process and provide much shorter converting times and reprinting times when compared with the state of the art, however at the same time showing sufficient paper and print quality e.g. gloss and print gloss.

Conventionally, in offset printing processes, always either irradiative drying (IR, UV), heat drying on the sheet fed press, an overprint varnish or so-called offset powders are routinely used in the printing process. The latter powders, which are also called anti setoff powders, anti-offset powders, dust, offset powder, powder and spray powder, are fine powders which are lightly sprayed over the printed surface of coated paper as sheets leave a press. These powders are therefore used in printing operations to facilitate the subsequent drying of inks. They are basically used to prevent the ink from transferring to the back side of the next sheet. When sprinkled over the printed surface, it prevents the front or printed side of a substrate from intimately contacting the back or unprinted side of a substrate. The starch particles act as spacers so air can enter from the sides and between the front and back of the substrate. This free flow of air across the inked surface allows inks that "dry" or cure by surface oxidation to receive exposure to oxygen in the air. The ink then cures to its final oxidized state.

Offset powder therefore obviously plays a very important role in a converting application that uses inks requiring oxidation to reach their final properties. Although offset powders are very beneficial, they can contribute detrimental characteristics. In applications in which a printed substrate is subject to further converting when perfect surface appearance is a requirement, use of offset powders may not be appropriate. E.g. in case of a printed substrate that will undergo lamination with an adhesive to a clear film. The application may be a label on which gloss and an optically perfect appearance are necessary. The dusting of offset powder acts like a sprinkling of dirt or other contaminant: It will produce surface imperfections in the laminate and seriously detract from the final appearance. They become entrapped in the lamination and contribute a "hills-and-valleys" appearance. This may be on a very small scale, but it is often enough to lead to an unsatisfactory appearance on close inspection. Another application in which the use of offset powder may not be appropriate is on a printed substrate used to make labels for the in-mould label process. In this process, a label printed on a paper or plastic substrate becomes an integral part of an injection- or blow-moulded container during the moulding operation. For the popular "no-label" look, the optical characteristics must be such that the consumer cannot see the label under any circumstances. Specks of offset powder, dust, or anything similar would detract from the appearance of such a label and make it unsatisfactory.

Nevertheless, so far the use of such offset powders (or of at least one of the other means as given above for supporting the ink drying) has always been regarded as unavoidable. Surprisingly it has now been found that in complete contrast to the expectations of the person skilled in the art, who would never have expected that this would be possible at all, we have now discovered that the use of such offset powders can be completely avoided and correspondingly the problems associated with such powders and to also avoid the necessity of any other drying step like infrared drying or heat drying or overprint varnish.

The present invention correspondingly proposes a printing sheet for sheet-fed offset printing with an image receptive coating layer on a paper substrate, which is characterised in that the printing sheet can be printed in an offset printing process without spraying a fine powder on the sheet as it comes off the press to prevent the ink from transferring to the back side of the next sheet. Also drying aids like heat or irradiation with infrared or UV or the use of overprint varnishes are not necessary any more.

According to a first preferred embodiment of the present invention, such a printing sheet is characterised by a particularly quick set off behaviour if printed with standard sheet fed offset inks. Such a paper preferably has a set off value of less than 0.4 measured 15 seconds after printing, which is a value that is far below the value of any commercially available offset printing papers. Even more preferred are set off values of less than 0.05, or even of less than 0.025 measured 15 seconds after printing.
Quantified differently or alternatively, such a printing sheet has a set off value of less than 0.05 measured 30 seconds after printing, preferably a set off value of less than 0.01 measured 30 seconds after printing.

It is however not only the drying property of the ink on a short timescale as quantified in the set of value which is important for avoiding the use of offset powders, it is also the drying property of the ink on a longer timescale. According to an other embodiment therefore the printing sheet is characterised by a multicolour ink setting value of less than 0.04 measured two minutes after printing. Preferably, it has a multicolour ink setting value of less than 0.02, preferably of less than 0.015 measured two minutes after printing.

Again quantified differently or alternatively, such a printing sheet has a multicolour ink setting value of less than 0.01 measured six minutes after printing, preferably of less than 0.005 measured six minutes after printing.

According to a particularly preferred embodiment of the present invention, the complete elimination of the use of offset powder is made possible by a printing sheet which has an appropriate balance of short a time ink setting properties avoiding problems induced by too quick absorption of the ink and corresponding possible rupture of the internal structure of the paper in the printing process, and of the longer time ink setting properties. This is possible by providing a printing sheet which has a set off value of less than 0.05, preferably of less than 0.02 measured 15 seconds after printing and a that it has a multicolour ink setting value of less than 0.04 measured two minutes after printing.

According to another preferred embodiment, the printing sheet is characterised in that a top coat and/or a second layer beneath it comprises a chemical drying aid, preferably selected from a catalytic system like a transition metal complex, a transition metal carboxylate complex, a manganese complex, a manganese carboxylate complex and/or a manganese acetate or acetylacetate complex (e.g. Mg(II)(Ac)₂ · 4 H₂O and/or Mn(acac)), wherein for proper catalytic activity of Mn complexes preferably Mn(II) as well as Mn(III) are present concomitantly, or a mixture thereof, wherein this chemical drying aid is preferably present in 0.5 to 3 parts in dry weight, preferably in 1 to 2 parts in dry weight. In case of a metal catalyst system like the above mentioned Mn complexes, the metal part of the catalyst system is preferably present in the coating in 0.05 - 0.6 weight-%, preferably in 0.02 - 0.4 weight-%, of the total dry weight of the coating. To support or enhance the catalytic activity of such systems is possible to combine them with secondary dryers and slash more auxiliary dryers. It is also possible to enhance the catalytic activity by providing different ligands for a metal systems, so for example the above acetate complex may be mixed with bipyridine-ligands (bipy). Also possible is the combination with other metal complexes like Li(acac). Further enhancements are possible by combining the catalytic systems with peroxides to have the necessary oxygen directly at the spot without diffusional limitations. It has to be pointed out that the use of such catalyst systems for fixing polymerizable or crosslinkable constituents of the offset ink is also advantageous for coatings of completely different nature and is not necessarily linked to the concept of having silica in a coating.

It can be shown that e.g. lower pigment contents (like silica) which have a specific porosity and/or specific surface and metal content can be compensated or even eliminated by the presence of such a chemical drying aid in the layer of the coating, and even a synergistic effect can be seen if the combination of silica and for example manganese acetate is used. The use of such a chemical drying aid in addition provides a further parameter to adjust the balance between paper gloss, print gloss, ink setting on a short timescale and ink setting on a longer timescale etc.

According to a further preferred embodiment, the printing sheet is provided with an image receptive coating layer which comprises a top layer and/or at least one second layer below said top layer, said top and/or second layer comprising: a pigment part, wherein this pigment part comprises a fine particulate carbonate and/or a fine particulate kaolin and/or a fine particulate silica and/or a fine particulate plastic pigment or a mixture thereof, at least one of its constituents with a surface area in the range of 18 or 40-400 m²/g or 100-400 m²/g, preferably in the range of 200-350 m²/g, and a binder part, wherein this binder part is composed of binder and additives. The specific surface area provides the advantageous quick ink setting necessary for the inventive concept. According to another preferred embodiment, the silica has a pore volume above 0.2 ml/g, preferably above 0.5 ml/g, even more preferred above 1 ml/g. In particular in combination with a fine particulate carbonate and/or kaoline and/or silica with a particle size distribution chosen such that the average particle size is in the range of 0.1-5 µm, preferably in the range of 0.3-4 µm the ink setting properties are optimal. Particularly good results can be achieved if the average particle size of silica is in the range of 0.3-1 µm or in the range of 3-4 µm. Also the surface properties of the silica used as well as its porosity have an influence on the chemical drying properties. Correspondingly, a fine particulate silica with a surface area in the range of 200-400 m²/g is preferred.

It is further noted that also the mentioned types of inorganic pigments (silica, ground and/or precipitated carbonates and/or kaolines) are able to contribute even more to the ink drying if they not only have surface area in the range of 40 or 100-400 m²/g, but if they in addition to that comprise traces of metal selected from the group of iron, manganese, cobalt, chromium, nickel, zinc, vanadium or copper or another transition metal, wherein at least one of these traces is present in an amount higher than 10 ppb or preferably higher than 100 or 500ppb or the sum of the traces is present in an amount higher than 100 ppb or preferably higher than 500ppb. The inorganic pigments may be intentionally or naturally enriched in such metal traces. E.g. an iron content above 500 ppb is preferred and if need be additionally a manganese content above 20 ppb. Also preferred is a chromium content above 20 ppb. This aspect of the presence of specific metal contents is actually also independent of the concept of a coating with silica.

The metal, be it in elemental or in ionic form, seems to contribute to the chemical drying of the ink. A larger content in metal may compensate a lower presence in parts in dry weight of pigment with the proper porosity and/or surface area, so for example if the pigment part comprises 80 - 95 parts in dry weight of a fine particulate carbonate and/or of a fine particulate kaoline, and 6 to 25 parts in dry weight of a fine particulate silica, the silica content may be smaller if it has higher metal contents.

There is 3 groups of metals which are particularly active as drier metals or related to drier function if present in one of the pigments, in particular in the silica fraction:
A) Primary or top or surface drier metals: all transition metals like Mn with both +2 (II) and +3 (III) valency. They catalyse formation and especially decomposition of peroxides, formed by reaction of O₂ with drying oils. This oxidative or free-radical chemistry leads to the formation of polymer-to-polymer crosslinks (= top drying) and also to formation of hydroxyl/carbonyl/carboxyl groups on the drying oil molecules. The most important ones are: Co, Mn, V, Ce, Fe. Also possible are Cr, Ni, Rh and Ru.
B) Secondary or through or coordination drier metals: The O-containing groups are used by these driers (but always in combination with primary driers, via joined complex formation) to form specific cross-links. The most important ones are: Zr, La, Nd, Al, Bi, Sr, Pb, Ba.
C) Auxiliary drier metals or promoter metals: they themselves do not perform a drying function directly, but via special interaction with primary or secondary driers (or some say via increase of solubility of prim. and sec. driers) they can support their activity. The most important ones are Ca, K, Li and Zn.
   To have significant activity of these metals, they should be present in the pigment (preferably in the silica) from 10 ppb as lower limit up to the following upper limits:
   Primary drier metals: all up to 10 ppm, except Ce: up 20 ppm.
   Secondary drier metals: all up to 10 ppm, except Zr,Al, Sr and Pb: here all up to 20 ppm.
   Auxiliary drier metals: all up to 20 ppm.

Some specific combinations of these metals are particularly effective, like e.g. Co + Mn, Co + Ca + Zr or La or Bi or Nd, Co + Zr/Ca, Co + La. Possible is e.g. a combination of Mn(II+III)acetate (only surface of ink is quickly dried and closed towards oxygen) with some K-salt (to activate Mn activity) and possibly with Zr-salt (to increase through drying of ink bulk, so to improve wet ink rub behaviour of printed ink layer).

A specific coating composition comprising silica is particularly advantageous according to the invention. Such an image receptive coating layer is designed such that it comprises a top layer and/or at least one second layer below said top layer, said top and/or second layer comprising: a pigment part, wherein this pigment part is composed of 80-95 parts in dry weight of a fine particulate carbonate (precipitated or ground carbonate or combinations thereof) and/or of a fine particulate kaolin, and 6 to 25, preferably 6 to 20 parts in dry weight of a fine particulate silica, and a binder part, wherein this binder part is composed of: 5-15 or even up to 20 parts in dry weight of binder and less than 4 parts in dry weight of additives. In this context it should be noted that the term particulate silica shall include compounds commonly referred to as silica sol, as well as colloidal silica, and also amorphous silica gel.

In a another preferred embodiment of the present invention, the pigment part comprises 7 - 15 preferably 8-12 parts in dry weight of a fine particulate silica, preferably 8 - 10 parts in dry weight of a fine particulate silica. As a matter of fact, if the silica content is too high, the printing ink shows ink setting which is too fast leading to inappropriate print gloss properties and other disadvantages. Therefore only a specific window of the silica content actually leads to appropriate properties for sheet fed offset printing, which requires a medium fast ink setting on a short timescale (in the range of 15-120 seconds as determined in the so-called set off test) but exceptionally fast ink setting on a long timescale (in the range of 2-10 minutes as determined in the so-called multicolour ink setting test).

According to another preferred embodiment of the invention, the pigment part comprises 70 - 80 parts in dry weight of a fine particulate carbonate, preferably with a particle size distribution such that 50% of the particles are smaller than 1 µm. Particularly good results can be achieved if a particle size distribution such that 50% of the particles are smaller than 0.5 µm is chosen, and most preferably with a particle size distribution such that 50% of the particles are smaller than 0.4µm.

As already pointed out above, the combination of carbonate and kaoline in the pigment part shows to have advantages. In respect of the kaoline it is preferred to have 10-25 parts in dry weight of a fine particulate kaolin, preferably 13- 18 parts in dry weight of a fine particulate kaolin. The fine particulate kaolin may be chosen to have a particle size distribution such that 50% of the particles are smaller than 1µm, even more preferably with a particle size distribution such that 50% of the particles are smaller than 0.5 µm, and most preferably with a particle size distribution such that 50% of the particles are smaller than 0.3 µm.

As already mentioned above, it is key to find a compromise between paper gloss and print gloss and fast ink setting properties. The faster the ink setting properties, the less advantageous usually the print gloss properties. Therefore a specific combination of binder proportion and silica proportion provides the ideal compromise for sheet fed offset printing without offset powder or the other means given above. Even better results can however be achieved if the binder part comprises 7 - 12 parts in dry weight of a binder. The binder may be chosen to be a single binder type or a mixture of different or similar binders. Such binders can for example be selected from the group consisting of latex, in particular styrene-butadiene, styrene-butadiene-acrylonitrile, styrene-acrylic, in particular styrene-n-butyl acrylic copolymers, styrene-butadiene-acrylic latexes, acrylate vinylacetate copolymers, starch, polyacrylate salt, polyvinyl alcohol, soy, casein, carboxymethyl cellulose, hydroxymethyl cellulose and copolymers as well as mixtures thereof, preferably provided as an anionic colloidal dispersion in the production. Particularly preferred are for example latexes based on acrylic ester copolymer which are based on butylacrylate, styrene and if need be acrylonitrile. Binders of the type Acronal as available from BASF (Germany) or other type Litex as available from PolymerLatex (Germany) are possible.

In addition to the actual binder, the binder part may comprise at least one additive or several additives selected from defoamers, colorants, brighteners, dispersants, thickeners, water retention agents, preservatives, crosslinkers, lubricants and pH control agents or mixtures thereof.

More specifically, a particularly suitable formulation for the application in sheet fed offset could be shown to be characterised in that the top coat of the image receptive layer comprises a pigment part, wherein this pigment part is composed of 80-95 parts in dry weight of a fine particulate carbonate and of a fine particulate kaolin 6 to 25 parts in dry weight of a fine particulate silica. Even better results can be obtained if the printing sheet is characterised in that the top coat of the image receptive layer comprises a pigment part comprising 70-80 parts in dry weight of a fine particulate carbonate with a particle size distribution such that 50% of the particles are smaller than 0.4µm, 10-15 parts in dry weight of a fine particulate kaoline with a particle size distribution such that 50% of the particles are smaller than 0.3µm, 8-12 parts in dry weight of a fine particulate silica with an average particle size between 3-5 µm and a surface area of 300-400 m²/g, and a binder part comprising 8-12, preferably 9-11 parts in dry weight of a latex binder less than 3 parts in dry weight of additives.

The printing sheet according to the present invention may be calendered or not, and it may be a matt, glossy or also a satin paper. The printing sheet may be characterised by a gloss on the surface of the image receptive coating of more than 75 % according to TAPPI 75deg or of more than 50 according to DIN 75deg for a glossy paper (e.g. 75-80% according to TAPPI 75deg), by values of less than 25% according to TAPPI 75deg for matt papers (e.g. 10-20%) and by values inbetween for satin grades (for example 25-35%).

An image receptive coating may be provided on both sides of the substrate, and it may be applied with a coat weight in the range of 5 to 15 g/m² on each side or on one side only. The full coated paper may have a weight in the range of 80 - 400 g/m². Preferably the substrate is a woodfree paper substrate.

Silica may be present in the top layer, it may however also be present in a layer which is right beneath a top layer. In this case, the top layer may also comprise silica, is however also possible to have a top free of silica. According to another preferred embodiment of the invention, the printing sheet is therefore characterised in that the image receptive coating layer has a second layer beneath said top layer comprising: a pigment part, wherein this pigment part is composed of 80- 98 parts in dry weight of a mixture of or a single fine particulate carbonate, preferably with a particle size distribution such that 50% of the particles are smaller than 2µm, 2-25 parts in dry weight of a fine particulate silica and a binder part, wherein this binder is composed of: less than 20 parts in dry weight of binder, preferably 8-15 parts in dry weight of latex or starch binder, less than 4 parts in dry weight of additives. In this case, it chose to have advantages if in this second layer the fine particulate carbonate of the pigment part consists of a mixture of one fine particulate carbonate with a particle distribution such that 50% of the particles are smaller than 2 µm, and of another fine particulate carbonate with a particle distribution such that 50% of the particles are smaller than 1 µm, wherein preferentially those two constituents are present in approximately equal amounts. Typically, the pigment part of the second layer comprises 5-15 parts in dry weight of silica, preferably in a quality as defined above in the context of the top layer.

It has to be pointed out that also further layers beneath such as second layer, which is optional, maybe provided. Such further layers may for example be sizing layers, there may however also be further layers even comprising certain amounts of silica. Preferably however, there is not more than two layers on the raw paper substrate, as it has been found that the set off behaviour of the paper is sometimes negatively influenced by the presence of two additional layers beneath the top player. Preferably therefore the paper is a double coated paper and not a triple coated paper.

As already discussed further above, the time to converting and reprinting should be reduced significantly. According to another preferred embodiment therefore the printing sheet is characterised in that it is re-printable and convertable within less than one hour, preferably within less than 0.5 hours.

The present invention furthermore relates to a method for making a printing sheet according as discussed above. The method is characterised in that a preferably silica comprising coating formulation is applied onto an uncoated, a precoated or on coated paper substrate, preferably on woodfree basis, using a curtain coater, a blade coater, a roll coater, a spray coater, an air knife, cast coating or specifically by a metering size press. Depending on the paper a gloss to be achieved, the coated paper may be calendered. Possible calendering conditions are as follows: calendering at a speed of in the range of 200-2000 m/min, at a nip load of in the range of 50 or 100-500 N/mm and at a temperature above room temperature, preferably above 60°C, even more preferably in the range of 70 - 95° Celsius, using between 1 and 15 nips.

Furthermore, the present invention relates to the use of a printing sheet as defined above in a sheet fed offset printing process without use of setoff powder and/or without irradiative or heat drying and/or without use of overprint varnish. In such a process preferably reprinting and/or converting takes place within less than one hour, preferably within less than 0.5 hours.
Further embodiments of the present invention are outlined in the dependent claims.

### SHORT DESCRIPTION OF THE FIGURES

In the accompanying drawings preferred embodiments of the invention are displayed in which are shown:
- Figure 1: a schematic cut through a coated printing sheet;
- Figure 2: grammage and thickness of middle coated papers;
- Figure 3: paper gloss of middle coated papers;
- Figure 4: paper roughness of middle coated papers;
- Figure 5: grammage and thickness of top coated papers - uncalendered;
- Figure 6: brightness and opacity of top coated papers - uncalendered;
- Figure 7: paper gloss level of top coated papers - uncalendered;
- Figure 8: ink setting of top coated papers - uncalendered, a) top side, b) wire side;
- Figure 9: practical print gloss vs. paper gloss of top coated papers - uncalendered;
- Figure 10: print snap of top coated papers - uncalendered;
- Figure 11: offset suitability of top coated papers - uncalendered;
- Figure 12: droplet test of top coated papers - uncalendered;

- Figure 13: wet ink rub resistance measured of top coated papers - uncalendered;
- Figure 14: grammage and thickness of top coated papers - calendered;
- Figure 15: brightness and opacity of top coated papers - calendered;
- Figure 16: paper gloss level of top coated papers - calendered;
- Figure 17: ink setting of top coated papers - calendered, a) top side, b) wire side;
- Figure 18: practical print gloss vs. paper gloss of top coated papers - calendered;
- Figure 19: print snap of top coated papers - calendered;
- Figure 20: offset suitability of top coated papers - calendered;
- Figure 21: droplet test of top coated papers - calendered;
- Figure 22: wet ink rub resistance measured of top coated papers - calendered;
- Figure 23: white gas test carried out in laboratory on calendered papers;
- Figure 24: ink scuff results of printed papers - uncalendered;
- Figure 25: mottle evaluations of uncalendered papers;
- Figure 26: ink scuff results of printed papers - calendered;
- Figure 27: mottle evaluations of calendered papers;
- Figure 28: white gas test results of calendered papers;
- Figure 29: wet ink rub resistance test results of calendered papers;
- Figure 30: set off values for top-side (a) and wire side (b) of calendered papers;
- Figure 31: multi colour ink setting values for top-side (a) and wire side (b) of calendered papers;
- Figure 32: offset suitability and MCFP for calendered papers;
- Figure 33: wet ink rub test results for calendered papers;
- Figure 34: Mercury intrusion porosity data of final coatings - coated papers; and
- Figure 35: particle size distributions of used pigments.

### DETAILED DESCRIPTION OF THE PREFERRED EMBODIMENTS

Referring to the drawings, which are for the purpose of illustrating the present preferred embodiments of the invention and not for the purpose of limiting the same, figure 1 shows a schematic view of a coated printing sheet. The coated printing sheet 4 is coated on both sides with layers, wherein these layers constitute the image receptive coating. In this particular case, a top coating 3 is provided which forms the outermost coating of the coated printing sheet. Beneath this top layer 3 there is provided as second layer 2. In some cases, beneath this second layer there is an additional third layer, which may either be a proper coating but which may also be a sizing layer.

Typically a coated printing sheet of this kind has a base weight in the range of 80 - 400 g/m², preferably in the range of 100-250 g/m². The top layer e.g. has a total dried coat weight of in the range of 3 to 25 g/m², preferably in the range of 4 to 15 g/m², and most preferably of about 6 to 12 g/m². The second layer may have a total dried coat weight in the same range or less. An image receptive coating may be provided on one side only, or, as displayed in figure 1, on both sides.

The main target of this document is to provide a coated printing sheet for "instant" ink drying for sheet fed-offset papers in combination with standard inks. Pilot coated papers were printed on a commercial sheet-fed press and ink setting as well as ink drying tests were carried out.

It was possible to speed up ink setting tendency of coated papers by use of silica (Syloid C803 and others like Sylojet, by Grace Davison) in second or top coating significantly compared to standard coated papers. For calendered papers a much better (faster) ink drying behaviour compared to uncalendered papers was observed. Improvements analysed via white gas test (also called benzin test) were confirmed by converting tests at practical printer (sheet-fed press).

Use of silica in top coating led to fast chemical drying, short time ink setting was also faster and mottle tendency of calendered paper even slightly better than for referent paper. Paper gloss and print gloss levels were slightly lower than reference.

When silica was used in the second coating, influence on chemical ink drying of the final paper still existed but the mechanism was not as active as for top coating application. Advantages of silica containing middle or second coating were higher paper gloss and equal ink setting time compared to reference which led to higher print gloss. For use in second coating silica amount had to be higher which resulted also in a higher product price of end paper.

Table 1 shows the different test papers which were used for the subsequent analysis. Five different papers were are made wherein the paper designated with IID_1 comprises a top coating without silica and a middle coating with silica, IID_2 comprises a top coating with silica and a middle coating without silica, IID_3 comprises no silica in standard middle coating or top coating, and IID_5 comprises a standard middle coating without silica and a top coating with silica. The detailed formulations of the middle coating and the top coating are given in tables 2 and 3 below.

**Table 1: trial plan (IID - for Instant Ink Drying) (B for middle coated papers)**

| | **IID_1** | **IID_2** | **IID_3** | **IID_5** |
|---|---|---|---|---|
| **Middle coat coating nr** | Blade MC_1 | Blade MC2 | | |
| coating weight WS [g/m²] | 11 | 11 | | |
| moisture [%] | 4.9 | 4.9 | | |
| coating weight TS [g/m²] | 11 | 11 | | |
| moisture [%] | 5.2 | 5.2 | | |
| **Top coat coating nr** | Blade TC_1/A | Blade TC_3/A | Blade TC_1/B | Blade TC_3/B |
| coating weight WS [g/m²] | 10.5 | 10.5 | 10.5 | 10.5 |
| moisture [%] | 4.9 | 4.9 | 4.9 | 4.9 |
| coating weight TS [g/m²] | 10.5 | 10.5 | 10.5 | 10.5 |
| moisture [%] | 5.0 | 5.0 | 5.0 | 5.0 |
| Coating weight total [g/m²] | 43 | 43 | 21 | 21 |
| | | | | |
| Printing trial | Paper 12 | Paper 11 | Paper 15 | Paper 13 |

**Table 2 Formulations of middle coatings**

| | Standard middle -coating | | MC_1 | | MC_2 |
|---|---|---|---|---|---|
| *Pigments* | % | *Pigments* | % | *Pigments* | % |
| HC 60 | **85** | HC60 | **40** | HC 60 | |
| HC 60 | **15** | | | | |
| HC 90 | | | | HC 95 | **100** |
| | | CC 60 | **50** | | |
| | | Syloid C803 | **10** | | |
| | | | | | |

| *Binders* | | *Binders* | | *Binders* | |
|---|---|---|---|---|---|
| Latex | **5** | Latex | **10** | Latex | **7.5** |
| Dextrin | **6** | Dextrin | **3** | Dextrin | **3** |
| | | | | | |

| *Additives* | | *Additives* | | *Additives* | |
|---|---|---|---|---|---|
| CMC | 0.3 | CMC | 0.4 | CMC | 0.3 |
| Polysalz S Plus others | 0.2 | Polysalz S Plus others | 0.2 | Polysalz S Plus others | 0.2 |

Remarks: MC_1 formulation is optimised in a way to reach fast long time ink setting by changes in middle coating- CC 60 (steep particle size distribution) is used to create higher pore volume silica as acceleration additive for chemical ink drying starch has also negative influence on pore volume - slows down long time ink setting but starch is also necessary as an rheology additive to increase water retention of coating colour if silica were to be replaced by additional 10% HC60 latex amount would be 7,5pph (clearly lower). Binding power: 10+ 0,5 * 3= 11,5. Binding power reference: 5+ 0,5 * 6=8.

MC_2 formulation is optimised based on practical experiences, where a fine pigment HC95 is used. Binding power: 7,5+ 0,5 * 3= 9

For both middle coating colours further additives are used as necessary (e.g. CMC, brighteners, rheology modifiers, defoamers, colorants etc.).

Middle coating colour MC_1 (with 10 % silica) and MC_2 (100% HC 95) were applied on a pre-coated paper (produced for 150 gsm). Starch level of middle coatings was reduced to 3 pph to reach fast ink setting - for common standard middle coating formulation 6 pph starch were used.

**Table 3 Top coating formulations**

| **Middle coat:** | | MS_1 | MS_2 | B middle coated | B middle coated |
|---|---|---|---|---|---|
| | | D1/A | D3/A | D1/B | D3/B |
| **Top coat:** | | TC_1/A | TC_3/A | TC_1/B | TC_3/B |
| | | IID_1 | IID_2 | IID_3 | IID_5 |

| | solid [%] | | | | |
|---|---|---|---|---|---|
| *Pigments* | | | | | |
| HC 60 | 78 | 3 | | 3 | |
| HC 90 | 76.5 | 15 | | 15 | |
| HC 95 | 78 | | | | |
| CC60 | 72 | | | | |
| Pigment SFC | 72 | 72 | 77 | 72 | 77 |
| Pigment Syloid C803 | 98 | | 8 | | 8 |
| Amazon | 72 | 10 | 15 | 10 | 15 |
| | | | | | |

| *Binder*/*Additive* | | | | | |
|---|---|---|---|---|---|
| Latex Acronal | 50 | 6.5 | 8.5 | 6.5 | 8.5 |
| Latex | 50 | 1 | 1 | 1 | 1 |
| CMC | 93.5 | 0.5 | 0.5 | 0.5 | 0.5 |
| PVOH | 20 | 1.2 | 1.2 | 1.2 | 1.2 |
| Fluocast | 50 | 0.55 | 0.55 | 0.55 | 0.55 |
| Polysalz S | 45 | 0.1 | 0.1 | 0.1 | 0.1 |

Two different top coating colours (TC_1 and TC_3) were prepared and applied on middle coated papers (produced for 150 gsm) as well as TC_1 (Standard) on MC_1 and TC_3 with 8% silica on MC_2 too.

Aims were an investigation of best coating layer for use of silica and to compare them with Standard coating (IID_3).

Middle and top coating application was done via blade coater (wire side was coated first) - coating weights, drying temperatures and moisture contents were chosen as commonly used.

Laboratory investigations of these coated papers were carried out using standard methods. Nevertheless, in view of the analysis of ink setting properties certain specific methods were used which shall be defined below:

### Wet ink rub test:

Scope: The method describes the evaluation of the rub resistance of papers and boards at several time intervals after printing, before full drying. Normative References / Relating International Standards: GTM 1001: Sampling; GTM 1002: Standard Atmosphere for Conditioning; ESTM 2300: Prüfbau printing device-description and procedure. Relating Test methods descriptions: Prüfbau manual.

### Definitions:

- Ink-rub: when submitted to mechanical stress like shear or abrasion, ink layers can be damaged and cause markings on the printed products, even if they are fully dried.
- Chemical drying: in sheet fed offset, the hardening of the ink film via reactions of polymerisation.
- Wet ink rub value: measurement of the amount of ink that has marked the counter paper during the wet ink rub test at a given time after printing.

Principle: A test piece is printed with commercial ink at the Prüfbau printing device. After several time intervals, a part of the printed test piece is rubbed 5 times against a blank paper (same paper). The damaging of the print and the markings on the blank paper are evaluated and plotted against a time scale. Printing ink Tempo Max black (SICPA, CH) is used.

Laboratory procedure: 1. Adjust the printing pressure to 800N, 2. Weigh the ink with a tolerance of 0,01g and apply the amount of ink on the inking part of the Prüfbau printing device, 3. Distribute the ink for 30s, (the ink distribution time can be lengthened to 60s for easier manipulation), 4. Fix the test piece on the short sample carrier, 5. Place the aluminium Prüfbau reel on the inking part and take off ink for 30s, 6. Weigh the inked reel (m₁), 7. Put the inked aluminium Prüfbau reel on a print unit, 8. Put the sample plate against the inked aluminium reel, print the test piece at 0.5m/s, 9. Mark the time at which the sample as been printed, 10. After printing, weigh again the inked reel (m₂) and determine the ink transfer Iₜ in g (Note: the ink transfer Iₜ is given by It = m₁-m₂ where m₁ is the weight of the inked reel before printing and m₂ the weight of the same reel after printing), 11. Adjust the number of rubbing on the Prüfbau ink rub resistance tester to 5, 12. Cut a round piece in the printed strip with the Prüfbau piece cutter. 13. Stick the test piece against one of the Prüfbau test piece carrier, and fix a blank strip of the same paper on the paper carrier, 14. After a defined time interval after printing, place the blank paper and the printed round piece face to face on the Prüfbau device and start the rubbing (five times), 15. Recommence the operation for all defined time intervals after printing and then, evaluate the papers drying as a function of the density of markings on the blank paper / damaging of the printed paper.

The chart below provides an example for the amount of ink to be weighed for the printing and the times after printing at which the ink rub test can be performed:

| Grades | Ink amount | Rubbing times (min.) |
|---|---|---|
| Gloss | 0.30g | 15 / 30 / 60 / 120 / 480 |
| Silk / Matt | 0.30g | 30 / 60 / 240 / 360 / 480 |

Results evaluation: The results are both measured and evaluated visually. Visual evaluation: order all the tested blank samples from best to worse as a function of the amount of ink that has marked the blank paper. Measurement: with the Colour Touch device, measure the colour spectrum of the blank samples (light source UV excluded). Measure the colour spectrum of the untested white paper. The colour spectra of the tested samples have a peak of absorption at a defined wavelength, which is typical for the ink used (this is the colour of the ink). The difference of the reflectance factors at this wavelength between the tested sample and the white untested sample is an indication of the ink rub. With the SICPA Tempo Max Black, the peak wavelength is 575nm and $InkRub = {\left({R}_{sample}-{R}_{blank}\right)}_{575 nm}$

### Folding test:

Execution: Each sheet is folded twice (cross fold). The first fold is made with a buckle, the second fold is made by a knife. The sheets are folded at different time intervals after printing.
Evaluation: The folding test is evaluated by visual judgement of the folded sheets.
For the folding test, two markings are significant:
- Cross-fold: the ink from the printed area is folded against a blank area.
- Guiding-reels markings: at the reception of the folding machine (transport-band), two plastic reels guide the sheets. In this case, the sheets went out with a blank area up, whereas the other side was a litho. The guiding reels made distinct marks by pressure/carbonising.

### Multicolour ink setting (laboratory) and K+E counter test (printer):

Scope: This method describes the measurement of the ink setting (stack simulation) at high ink coverage of all papers and boards for offset printing. The high ink coverage is obtained by printing with multiple colours from 2 nips (laboratory) to 4 colours (commercial printing). This standard describes both laboratory and commercial printing standard tests.

### Definitions:

Set-off: ink transfer from a freshly printed paper to a counter paper (same paper) after different penetration times.

Counter paper: The counter paper absorbs the ink that has not set. In this test, the

counter paper is the same as the tested paper.

Setting value: density of the ink transferred to the counter paper.

Principle: A sheet is printed. After several time intervals, a part of the printed test piece is countered against the same blank paper. The density of the transferred ink of each area on the counter paper is measured and plotted against a time scale.

Preparation of test pieces: Mark the topside of the paper or board. Cut a test piece of approximately 4,6 cm x 25,0 cm. Sheet fed: For a sheet fed paper or board cut the longest side of the test piece parallel to the cross direction. Reel fed: For a reel fed paper or board cut the longest side of the test piece parallel to the machine direction. Cut the counter paper in pieces of approximately 4,6 cm x 25,0 cm (mark the contact-side of the paper).

Standard Procedure for laboratory, multicolour ink setting (MCIS): 1. Adjust the printing pressure of the 2 printing units to 800N, 2. Adjust the printing speed to 0.5m/s, 3. Weigh two sets of ink with a tolerance of 0.01 g and apply the 2 amounts of ink on 2 inking parts of the Prüfbau printing device, 4. Distribute the ink for 30s, (the ink distribution time can be lengthened to 60s for easier manipulation), 5. Fix the test piece to the sample carrier, 6. Place the 2 aluminium Prüfbau reels on the inking part and take off ink for 30s, 7. Weigh the 2 inked reels m₁₁ and m₂₁, 8. Put the 2 inked aluminium Prüfbau reels on the printing units, 9. Put the sample carrier against the first inked aluminium reel, print the test piece at 0.5m/s and switch on the stopwatch at the same time, 10. Weigh the 2 inked reels m₁₂ and m₂₂ after printing and calculate the ink transfer It in g given by: It = (m₁₂ - m₁₁) + (m₂₂ - m₂₁), 11. Clean the two aluminium Prüfbau reels, 12. Place the right (second) Prüfbau reel back on the printing unit, 13. Turn the FT 10 module on, 14. Put the test piece in front of the left (first) printing unit (no reel on this printing unit), 15. Set the time delay switch at about 2 seconds, 16. Press the start button on the FT 10 module, 18. After 1 minute and 53 seconds, press the start button of the FT10 module, 19. When the countering is done, remove the sample, turn the FT10 module off and switch the time delay back to 0s, 20. When the ink is dry, measure the density (McBeth) of the 3 areas (2, 6 and 10 minutes) on the counter paper. The density of one area is the average of ten measurements, which are taken according a pattern.

The time intervals that can be used for the MCIS test: 2 min, 6 min., 10 min.. until no marking.

Procedure for practical printing (K&E counter test, also "Heidelberg test"): 1. The pressure reels are on position "high" (hand-levers in position high), 2. Put the reels at the top extremity of the K&E setting equipment table, 3. When a freshly printed sheet is taken out of the press by the printer, start the stopwatch, 4. Lay the sheet flat on the K&E (also called "Heidelberg") setting equipment, with the printed side of the sheet above, 5. Place a blank sheet of the same paper flat on the printed sheet, bottom on top, 6. At the defined time interval, put the pressure reels on position "low" and drive the pressure reels to the opposite extremity of the K&E setting equipment table at constant speed, 7. Put the reels again in position "high" (hand-levers on position high) and drive the reels to their initial position (opposite extremity of the K&E setting equipment table), 8. Remove the counter sheet from the printed sheet, 9. Repeat the operation with a new fresh sheet and a new blank paper for all the time intervals defined.
The time intervals that can be used for the K&E test:15sec. 30sec. 60sec. 120sec. 180sec. until no marking.

### Set off test:

Scope: The set-off test method describes the measurement of the set-off (pile simulation) of all papers and boards used for sheet fed and reel fed offset printing. The counter paper used is the same as the paper tested.

### Definitions:

Ink penetration: phenomenon of selective absorption of the ink components into the paper.

Counter paper: The counter paper absorbs the ink that has not set.

Set-off: ink transfer from a freshly printed paper to a counter paper (same paper) after different penetration times.

Sett-off value: density of the ink transferred to the counter paper.

Principle: A sample is printed with a standard ink on the Prüfbau printing device. After several time intervals, a part of the printed sample is countered against a counter paper (top on bottom in order to simulate a pile). The density of the transferred ink of each area on the counter paper is measured and plotted against time.

Device: Prüfbau printing device; Aluminium Prüfbau reels 40 mm; Prüfbau sample carrier; Huber Setting Test Ink cyan 520068; Counter paper: same paper as tested paper; Gretag McBeth-densitometer (DC-type, with filter).

Procedure: 1. Adjust the printing pressure for both printing units to 800 N; 2. Adjust the switch for the waiting time to 2 seconds; 3. Adjust the printing speed to 0.5m/s; 4. Weigh the ink with a tolerance of 0.001 g and apply the amount of ink on the inking part of the Prüfbau printing device (Attention: different ink amounts for gloss and silk/matt grades); 5. Distribute the ink for 30s; 6. Fix the test piece on the sample carrier; 7. Place the aluminium Prüfbau reel on the inking part and take off ink for 30s, 8. Weigh the inked reel (ml); 9. Put the inked aluminium Prüfbau reel on the left print unit and the clean reel on the right countering unit; 10. Put the sample carrier against the inked aluminium reel, switch the printing speed on and switch on the stopwatch at the same time; 11. Switch the printing speed off; 12. Put the counter paper on top of the printed test piece (top on bottom); 13. Move the handle of the Prüfbau printing device up and down until the blanket of the sample carrier is against the clean aluminium Prüfbau reel; 14. Move the handle of the Prüfbau printing device up and down after 15, 30, 60 and 120s, while holding the counter paper vertically after the nip to avoid prolonged contact with the printed paper; 15. After printing, weigh the inked reel (m2) again and determine the ink transfer It in g wherein the ink transfer It is given by It = m1-m2 where m1 is the weight of the inked reel before printing and m2 the weight of the same reel after printing; 16. When the ink is dry, measure the density (Gretag-Mc Beth densitometer, cyan filter) of the areas (15, 30, 60 and 120s) on the counter paper, wherein the density of one area is the average of 10 measurements, which are taken according to a pattern.

### White gas test:

The white gas test is used to evaluate the time needed for a sheet fed offset ink film printed on a paper to be chemically dry.

Definitions: Chemical ink drying: full cross-linking of unsaturated vegetable oils of the ink via oxydopolymerisation.

Principle: A sample is printed with a standard commercial ink on the Prüfbau printing device. After several time intervals, a part of the printed sample is put in contact with white gas. The white gas can dissolve the ink film on the paper as long as the ink film is not totally cross-linked. When the white gas does not dissolve the ink film anymore, the sample is considered chemically dry.

Device: Prüfbau printing device; Aluminium Prüfbau reel 40 mm; Prüfbau sample carrier; Tempo Max Black (SICPA); FOGRA-ACET device.

Sampling and test piece preparation: For the white gas test, cut a piece of the strip of at least 5cm length. Then: 1. Adjust the pressure of the printing nip of the Prüfbau printing device to 800N; 2. Adjust the printing speed to 0.5m/s; 3. Weigh the ink with a tolerance of 0.005g and apply the amount of ink on the inking part of the Prüfbau printing device; 4. Distribute the ink for 30s; 5. Fix the test piece on the sample carrier; 6. Place the aluminium Prüfbau reel on the inking part and take off ink for 30s; 7. Put the inked aluminium Prüfbau reel on the right print unit; 8. Put the sample carrier against the inked aluminium reel and switch the printing speed on; 9. Switch the printing speed off; 10. Mark the time of printing (e.g.: starting time for the white gas test); 11. Choose the thickness card that corresponds to the paper's grammage; 12. Cut a piece of the strip of at least 5cm length; 13. Stick the extremity of the strip to the thickness card with tape; 14. Place a felt pad in the pad holder of the FOGRA-ACET device; 15. Pump 0.5ml white gas with the all glass syringe and apply it on the felt pad; 16. Place the thickness card with the sample to be tested in the card holder; 17. Close the FOGRA-ACET device and immediately pull the thickness card with the test sample attached to it out of the device; 18. Evaluate the chemical drying of the sample; 19.

Repeat the operation every hour until the sample is fully dry (no dissolving of the ink layer visible.
Calculations: The chemical drying time of a printed ink film is the time at which the ink on the sample tested could not be dissolved. The chemical drying time is given in hours.

### Droplet test (also called wet repellence test):

Definition: Wet repellence: Shows the influence of fountain solution on ink absorption. Principle: Before a strip of paper is printed with an aluminium reel, a drop of 20% Isopropyl Alcohol solution is applied on the paper. The drop will be spread by the printing reel between paper and ink. The higher the density of colour on the wetted area, the better the wet repellence.

Device: Prüfbau printing device; Aluminium Prüfbau reel 40 mm; Blanket Prüfbau sample carrier long; Huber picking test ink 408001; 20 (v/v)% Isopropyl alcohol-solution; Gretag-McBeth densitometer (DC-type, with filter);

Sampling and test piece preparation: Mark the topside of the paper or board. Cut a test piece of approximately 4,6 cm x 25,0 cm. For sheet fed and reel fed papers cut the longest side of the test piece parallel to the machine direction. Then: 1. Adjust the printing pressure for both printing units to 800N; 2. Adjust the printing speed to 1.0m/s; 3. Weigh the ink with a tolerance of 0.005g and apply the amount of ink on the inking part of the Prüfbau printing device (No different ink amounts for gloss and silk/matt grades); 4. Distribute the ink for 30s; 5. Fix the test piece on the sample carrier; 6. Place the aluminium Prüfbau reel on the inking part and take off ink for 30s; 7. Put the inked reel on the printing unit; 8. Put the sample plate against the inked reel; 9. Put with the pipette a drop of 5 µl 20% Isopropyl-alcohol on the paper; 10. Print the test piece immediately after setting the drop; 11. Remove the printed test piece from the sample plate; 12. After 24 hours the density of dry area ("dry-density") and the density of the wetted area ("wet-density") is measured.

Calculations: The wet repellence in percentage is calculated by dividing the wet density by the dry density and multiplying it by 100. The higher the value, the better the wet-repellence. Typically: < 20% very bad; 20-30 % bad; > 30 % good.

### Thumb test:

Non-standard; in line with general practice of commercial printing (and also in paint testing area) at several time intervals (15, 30, 60, 90 ....minutes) a thumb, covered with (special) house-hold tissue paper (to avoid influence of skin grease), is firmly (but always at about same force) pressed and simultaneously turned over 90° in the printed ink layer. In case of fully wet stage all ink is wiped off, leaving a clear white spot on paper substrate. In case of fully chemically dried ink no injury can be seen. It is preferred that one and the same operator is performing all series.

### Experimental Results, Part 1

Laboratory investigations of middle and top coated papers (uncalendered): Grammage and thickness of middle coated papers, paper gloss of middle coated papers, and paper roughness of middle coated papers are given graphically in figures 2-4, respectively, wherein the data designated with IID_4 are not the object of these investigations. Paper calliper and with it specific volume is higher for middle coated papers as produced on a standard paper machine. Paper gloss of middle coated papers MC_1 and MC_2 is clearly higher than those of middle coated papers. Main reason for this seems to be the use of coarse pigments (HC60) and higher starch level for current standard middle coating as used in IID_3, and IID_5. Highest gloss level is reached with MC_2 which has 100% HC95 in coating formulation. Measured PPS-values do not confirm observed gloss differences, as one can see from Figure 4. Grammage and thickness of top coated papers - uncalendered- are given in Figure 5. Paper grammage of top coated papers points out a variation from 144 gsm for IID_1 and IID_2 to 151 gsm for IID_5.

Brightness and opacity of top coated papers - uncalendered, as well as paper gloss level of top coated papers - uncalendered, are given in Figures 6 and 7, respectively. The highest paper gloss level is seen for papers with standard formulation, silica in top coating colour reduces paper gloss slightly (Tappi 75° ~ 10% and DIN 75° ~ 5%). Ink setting of top coated papers - uncalendered, and practical print gloss vs. paper gloss of top coated papers - uncalendered, are given in figures 8 and 9, respectively. Very rapid ink setting can be recognised for top coatings containing silica (see figure 8, wherein figure 8 a) displays the values for the topside and figure 8 b) the values for the wire side). On the other hand, also paper gloss and print gloss go down for those two samples (see figure 9, topside of uncalendered papers shown).
Figure 10 shows the print snap (print gloss minus paper gloss) of top coated papers - uncalendered, and figure 11 shows the offset suitability (passes until fail) of the top coated paper -uncalendered. Extremely fast ink setting is observed for papers IID_2 and IID_5 with silica in top coating colour - possible advantage for fine middle coating as used for IID_2. Slowest ink setting was measured for reference paper IID_3 ― use of silica in middle coating with standard top coating (TC_1) leads to faster ink setting. Extremely fast short time ink setting usually leads to lower print gloss at commercial printer. Highest print snap is measured for IID_1 ― lowest one for IID_2. The offset suitability of paper IID_2 shows to be approximately 2 passes lower than those of reference IID_3. Increase of latex in top coating colour TC_3 however leads to a reduced ink setting speed and to an increased print gloss level. The balance of these two constituents (silica, binder) therefore has to be chosen carefully in accordance with the needs in terms of print gloss etc.

As one can see from figure 12, extremely high droplet test values were measured for silica containing paper. Here, also an obvious influence of middle coating was observed. Fast short time ink setting and high absorption rate of paper IID_2 leads to good wet ink rub resistance (low value) measured in laboratory as one can see from figure 13 (wet ink rub resistance measured of top coated papers - uncalendered ; the lower the better).

### Experimental Results, Part 2

Laboratory investigations of top coated papers calendered: With reference paper roll IID_3 calendering setting was adjusted to reach gloss target DIN 75° (55%) and kept constant for all other rolls. The following parameters were chosen for calendering:
Speed: 300 m/min; Nip load: 290 N/mm; Temperature: 90°C; Nips used: 11.

Grammage and thickness of top coated papers - calendered - are given in figure 14, brightness and opacity of top coated papers - calendered - are given in figure 15, and paper gloss level of top coated papers - calendered - are given in figure 16.

Paper grammage and calliper of calendered papers are comparable. After calendering paper gloss differences are mainly damped - slightly higher values are measured for paper IID_1.

Figure 17 shows the ink setting of top coated papers - calendered, wherein a) shows the data for the topside and b) shows the data for the wire side. Again, strikingly and exceptionally low ink setting values can be observed for the two coatings IID_2 and IID_5 comprising silica in the top coating.

Practical print gloss vs. paper gloss of top coated papers - calendered - is given in figure 18, print snap (print gloss minus paper gloss) of top coated papers - calendered - is given in figure 19, and the offset suitability (passes till fail) of top coated papers-calendered - is given in figure 20.

Again extremely fast ink setting is observed for calendered papers IID_2 and IID_5 with silica in top coating colour - at this fast ink setting level some advantage for fine middle coating used for IID_2 is visible.

Slowest ink setting was measured for reference paper IID_3 ― use of silica in middle coating with standard top coating (TC_1) leads to faster ink setting.

General set-off value measured after 15 seconds is slower than for uncalendered papers (influence of paper smoothness) - after 30 seconds faster values for calendered papers (finer pores).

Extremely fast short time ink setting leads to lower print gloss at commercial printer.

Highest print snap is measured for reference IID_3 ― lowest one for IID_2.

Offset suitability of paper IID_2 is lower than those of reference IID_3. Increase of latex in top coating colour TC_3 leads to a reduced ink setting speed and as result to an increased print gloss level. Again, therefore, the balance of the two constituents of silica and latex binder can to be adjusted according to current needs.

Figure 21 shows the results of droplet test of top coated papers - calendered. Fast short time ink setting and high absorption rate of paper IID_2 and IID_5 lead to good wet ink rub resistance (low value) measured in laboratory even 5 minutes after printing, as one can see from figure 22, in which the wet ink rub resistance of top coated papers is graphically given.

White gas test carried out in laboratory (see figure 23, white gas test data) shows faster chemical drying for papers with silica in top coating.

### Experimental results, part 3, practical printing trials

Uncalendered as well as calendered papers were printed on a practical sheet-fed press to check possibilities for a glossy and silk paper development. Just the top side was printed.

### a) Uncalendered papers:

Figure 24 shows ink scuff results of printed papers - uncalendered (ink scuff is a term that is variably used by printers. Generally, one understands ink markings by ink scuff. Such ink markings can be produced by different causes: * if the ink is not fully dry → seen in wet ink rub test; * if the ink is fully dry → seen in ink rub resistance test. The wet ink rub test, which is a convertibility test, is detailed above. The ink rub resistance test shares the same principle as the wet ink rub test, but it is carried out after the ink has dried for 48 hours.)

Generally high (worse) ink scuff values of uncalendered papers measured at printer are observed - best level for paper IID_5 and worst level for reference IID_3.

Folding test evaluations given in table 4 below show lowest marking tendency at folding of a printed 300% area (against a blank area) for uncalendered paper IID_2 even after 0,5 hour after printing followed by paper IID_1 with good level 2 hours after printing. Paper IID_3 without silica is clearly worse at folding test.

The same trend is found for white gas test (also called benzin test) carried out at printer on a 400% printed area - paper IID_2 starts to get dry (chemically dry) after 3 hours, paper IID_5 after 4 hours, paper IID_1 after 5 hours but for reference paper IID_3 chemical drying was not observed until 24 hours have expired.

It can be summarised that clear improvements of chemical drying process by use of silica are confirmed by practical printing trials.

Mottle evaluations of uncalendered papers are given in figure 25. The results of a K+E counter test of printed paper (time till no countering was visible - the lower the better): $IID_ 1 = 240 minutes , IID_ 2 > 180 minutes , IID_ 3 > 300 minutes , IID_ 5 > 240 minutes ,$

### b) Calendered papers:

Figure 26 shows ink scuff results of printed papers - calendered. Much better (lower) ink scuff values measured at printer are observed for calendered papers compared to uncalendered papers with best level for paper IID_2 and worst level for reference IID_3.

Folding test evaluations given in table 5 below show lowest marking tendency at folding of a printed 300% area (against a blank area) for silica containing calendered papers IID_1, IID_2 and IID_5 even after 0,5 hour. Paper IID_3 without silica is clearly inferior in the folding test.

The same trend is found for white gas test carried out at printer on a 400% printed area - paper IID_2 starts to get dry (chemical dry) after 2 hours, papers IID_1 and IID_5 after 4 hours but for reference paper IID_3 chemical drying is observed not until 24 hours.

It can be summarised that clear improvements of chemical drying process by use of silica is confirmed by practical printing trials.

Tendency of laboratory coating tests show good correlation to observations at printer.

The best mottle tendency (lowers values) is observed for calendered papers IID_1 and IID_2 which had also very fast chemical drying behaviour.

Level of matt papers is clearly worse than the one of calendered papers.

Figure 27 shows the mottle evaluations of calendered papers. Results of the K+E counter test of printed paper (time till no countering is visible - the lower the better) are as follows: IID_1= 240 minutes; IID_2= 180 minutes; IID_3> 420 minutes; IID_5 > 360 minutes.
Caused by a smoother paper surface of the calendered papers higher ink transfer to counter paper takes place which leads to longer times till no countering is visible.

### Experimental results, part 4

In a further effort to specify the critical limits of the formulations, in a separate series of experiments the influence of the silica content in the coatings was evaluated. Prepared top coatings were applied on a Dow-coater on a regular paper substrate without topcoat layer, meant for 250 gsm end-paper i.e. on a substrate only with regular (not enhanced) middle coat composition. Silica amount (in this case Syloid C803) in top coating colour was increased from 0% (Standard top coating) up to 3% and 10% (see table 6 below).
For all coating formulations latex level was kept constant at a level of 8pph. Papers were calendered (2 passes with 2000 daN nip load and 75°C temperature of steel roll) and tested in laboratory.

**Table 6: Formulations of top coating, coating colour composition in %**

| Product / Trial-Nr. | SC | 20 | 21 | 23 |
|---|---|---|---|---|
| Setacarb HG | 75.0 | 100 | 100 | 100 |
| Litex | 50.0 | 8 | 8 | 8 |
| Starch | 25.0 | 0.4 | 0.4 | 0.4 |
| PVOH | 22.0 | 1.8 | 1.8 | 1.8 |
| Thickener | 30.0 | 0.024 | 0.024 | 0.024 |
| Polysalz S | 40.0 | | 0.1 | 0.1 |
| Syloid C803 | 99.4 | | 10 | 3 |
| | | | | |
| Based on pigment atro | | 500 | 500 | 500 |
| Solids | | 69.24 | 70.99 | 69.75 |

**Table 7: Experimental findings for the formulations 20, 21 and 23 according to table 6.**

| Product / Trial-Nr. | | | 20 | 21 | 23 |
|---|---|---|---|---|---|
| **Set off** | | | | | |
| Set-off 15 sec. | top | | 0.90 | 0.27 | 0.63 |
| | wire | | | | |
| Set-off 30 sec. | top | | 0.53 | 0.07 | 0.12 |
| | wire | | | | |
| Set-off 60 sec. | top | | 0.07 | 0.01 | 0.04 |
| | wire | | | | |
| Set-off 120 sec. | top | | 0.03 | <0,01 | 0.01 |
| | wire | | | | |

| **Wet Ink Rub** | | | | | |
|---|---|---|---|---|---|
| 15 min | top | | 1.78 | 1.45 | 2.69 |
| 30 min | top | | 6.43 | 0.77 | 9.2 |
| 60 min | top | | 3.1 | 0.74 | 8.44 |
| 120 min | top | | 3.05 | 0.7 | 5.27 |

| **Chemical Ink Drying** | | | | | |
|---|---|---|---|---|---|
| Thumb test | top | h | 3 | <1 | 1.5 |
| Thumb test | wire | h | | | |
| White gas test | top | h | >3,5 | 1 | 3.5 |
| White gas test | wire | h | | | |

| **Gloss (unprinted)** | | | | | |
|---|---|---|---|---|---|
| Gloss Tappi 75° | top | | 74.3 | 64.6 | 74.1 |
| | wire | | | | |
| Gloss DIN 75° | top | | 55.6 | 43.9 | 53.6 |
| | wire | | | | |
| Gloss DIN 45° | top | | 17.0 | 8.2 | 16.4 |
| | wire | | | | |

| **Gloss (printed as for ink drying test)** | | | | | |
|---|---|---|---|---|---|
| Gloss Tappi 75° | top | | 77.4 | 66.8 | 77.3 |
| | wire | | | | |
| Gloss DIN 75° | top | | 34.1 | 26.6 | 34.4 |
| | wire | | | | |
| Gloss DIN 45° | top | | 19.1 | 11.3 | 18.5 |
| | wire | | | | |

### Discussion of the results:

- Presence of less than 3 or 5 part of silica in this series does not lead to significant desired effect, so the inventive choice is clearly limited in its boundaries.
- Presence of 10 parts silica-gel Syloid C803 results in very fast physical ink-setting behaviour, according to (short time) set-off test and thumb test data. Also according expectations, this fast behaviour slows down in case of less amount Syloid C803.
- It is however quite surprising that presence of 10 parts Syloid C803 apparently also causes quite significant enhancement of ink chemical drying behaviour: white gas test dry in < 1 h.
- Potential drawbacks of Syloid C803 product, partly related to its fast physical ink-setting behaviour are its relatively low print gloss and paper gloss. Possible solutions for improved print gloss: more latex binder, see below part 5.
- Another further explanation for the intrinsic chemical drying potential of Syloid C803, apart from the surface properties and the porosity, seems to be presence of residual transition metals (out of raw material water glass) like Fe (60-70 ppm) and Co (< 0,2 mg/kg) on the surface of inner pores. Quite generally one can say, that a selective enrichment in transition metals of the silica used is be an possibility for further increasing the chemical drying effect of silica.

In respect of the last issue, further investigations were carried out to determine the actual content of these traces of metals. Elemental analysis of various commercially available silica was carried out using ICP, wherein the samples were prepared as follows: GASIL 23D: (1.0 g); GASIL 35M: (1.0 g); Ludox pw50: (5.0 mL); Sylojet 710A: (5.0 mL); Syloid C803: (1,0 g), were mixed with HNO₃ into an 50ml solution for ICP analysis. The values as given in table 8 were obtained.

It can be noted that the product Ludox, which is characterised in rather high metal 5 content, does not show satisfactory ink drying tendency. An explanation for this is the fact that this silica has almost no porosity and that it has a specific surface which is too small for the chemical drying to develop significant effect.

As already pointed out above, in principle not only silica could be used to produce the effect according to the invention, but also conventional pigments (for example 10 carbonates, kaoline) as long as they have a porosity, a particle size distribution and a specific surface as specified for the above silica, and as long as they comprise traces of metal in the same range as given in table 8.

### Experimental results, part 5

As pointed out above, the latex content can be used for slightly slowing down ink setting on a short timescale and for increasing the gloss. In order to show that the claimed range for the binder indeed is an inventive selection, a series of experiments was carried out to find out what the optimum latex content would have to be.

Paper substrate: Regular papers without topcoat layer, meant for 250 gsm end-paper quality. Latex level of silica containing (10%) coatings was increased stepwise 8 to 10 and 12 pph. Coating colours were applied via bird applicator (yield of the coating on the paper was 5 -7 gr → quite low but trend should be observable). Papers were calendered (2 passes with 2000 daN nip load and 75°C temperature of steel roll) and tested in laboratory.

**Table 9 Formulations for the evaluation of influence of Latex binder content**

| Coating Colour Composition in % | | | | | |
|---|---|---|---|---|---|
| | | Ref | 2 | 4 | Stand. |
| Product / Trial-Nr. | SC | 1 | 2 | 3 | 4 |
| Setacarb HG | 75,0 | 90 | 90 | 90 | 100 |
| Litex | 50,0 | 8 | 10 | 12 | 8 |
| Starch | 25,0 | 0,4 | 0,4 | 0,4 | 0,4 |
| PVOH | 22,0 | 1,8 | 1,8 | 1,8 | 1,8 |
| Thickener | 30,0 | 0,0 | 0,0 | 0,0 | 0,024 |
| Calciumstearat | 50,0 | 0,700 | 0,700 | 0,700 | |
| | 1 | | | | |
| Syloid C803 | 99,4 | 10,0 | 10,0 | 10,0 | |
| | | | | | |
| Based on pigment atro | | 250 | 250 | 250 | 250 |
| Solids | | 70,50 | 70,00 | 69,51 | 69,24 |
| Solids target A | | 60,00 | 60,00 | 60,00 | |

The results are summarised in table 10:

**Table 10 Results of the evaluation of influence of Latex binder content**

| Topcoat | Thumb dry | White gas dry | solids | Print gloss Tappi 75 | Print gloss Din 75 | Print gloss Din 45 |
|---|---|---|---|---|---|---|
| 1 | 1 h | 1-2 h | 60,0 % | 65.88 | 25.05 | 11.40 |
| 2 | 1 h | 1 h | 59,7 % | 74.17 | 33.16 | 17.77 |
| 3 | 2 h | 3 h | 60,5 % | 80.63 | 39.23 | 22.80 |
| 4 | 3-4 h | > 5 h | 68.9 % | 87.42 | 38.58 | 22.96 |

Set off and MCIS tests indicate that the drying behaviour is only slightly influenced by the latex content.
Conclusions:
- Short time ink setting (set off) is slightly slowed down by use of more latex (no significant additional difference for +2 and + 4 pph latex observed) but still faster than reference paper.
- Print gloss is increased, if more latex is added (caused by slower set off).
- Long time ink setting speed (multicolour ink setting) is also slightly decreased with more latex (slower than reference paper).
- Ink drying time (thumb test) does not increase, if 2pph extra latex is added.
- Adding 4 extra parts slows down ink drying, level obtained with +4 pph latex is still better than reference. Print gloss is comparable to reference (DIN 75 and DIN 45 values)

### Experimental results, part 6

The aim of this part is to determine an optimum concept for middle and top coatings with silica to improve chemical ink drying.

Experiment: Paper substrate: Regular papers without middle and top coating layer, meant for 250 gsm end paper. Prepared middle and top coatings were applied on Dow-coater (coated just on one side, pre coating application 12 gsm, top coating application 12 gsm). Papers were calendered (2 passes with 2000 daN nip load and 75°C temperature of steel roll) and tested in laboratory.

The trials according to Table 11 were carried out:

**Table 11 Trials for evaluation of middle coating**

| | | |
|---|---|---|
| Trial number | First coating layer | Second coating layer |
| | | |
| 45 | Precoat 2 | TC2 |
| 47 | Precoat 2 | TC6 |
| 48 | Precoat 3 | TC1 |
| 49 | Precoat 3 | TC2 |
| 50 | Precoat 3 | TC3 |
| 53 | Precoat 3 | TC6 |

The following formulations were used for the trials (see table 12):

**Table 12 Formulations for the trial according to experimental part 6.**

| | | Precoat 1 | Precoat 2 | Precoat 3 | TC1 | TC2 | TC3 | TC6 |
|---|---|---|---|---|---|---|---|---|
| | | | | | | | | |
| Product / Trial-Nr. | SC | 1 | 2 | 3 | 4 | 5 | 6 | 9 |
| Setacarb HG | 75.0 | | | | 100.0 | 95.0 | 90.0 | 90.0 |
| Hydrocarb 95 | 78.0 | 90.0 | 95.0 | 100.0 | | | | |
| Sylojet 703A | 19.3 | | | | | | | |
| Syloid C803 | 99.4 | 10.0 | 5.0 | | | 5.0 | 10.0 | 10.0 |
| Latex | 50.0 | 12.0 | 11.5 | 11.0 | | | | |
| Litex | 50.0 | | | | 8.0 | 8.0 | 8.0 | 10.0 |
| Starch | 25.0 | 1.0 | 1.0 | 1.0 | 0.4 | 0.4 | 0.4 | 0.4 |
| CMC | 20.0 | 0.3 | 0.3 | 0.3 | | | | |
| PVOH | 22.0 | 0.3 | 0.3 | 0.3 | 1.8 | 1.8 | 1.8 | 1.8 |
| Thickener | 30.0 | | | | 0.027 | 0.027 | 0.027 | 0.027 |
| Calciumstearate | 50.0 | 1.0 | 1.0 | 1.0 | 0.7 | 0.7 | 0.7 | 0.7 |
| | | | | | | | | |
| **Based on pigment atro** | | 500 | 700 | 1000 | 300 | 600 | 300 | 500 |
| Solids | | 72.39 | 71.90 | 71.42 | 69.07 | 69.78 | 70.50 | 70.00 |
| Solids target A | | 57.00 | 62 | 68 | 68 | 62 | 57 | 57 |
| Solids target B | | | | | | | | |
| Solids target C | | | | | | | | |

First applied coating layer is the middle or second coating; second applied coating layer is the top coating.

The results of the printing properties are summarised in table 13:

**Table 13 summary of the printing properties of experimental part 6**

| | | | Pre2+TC2 | Pre2+TC6 | Pre3+TC1 = Reference | Pre3+TC2 | Pre3+TC3 | Pre3+TC6 |
|---|---|---|---|---|---|---|---|---|
| | | | | | | | | |
| Set off | | | | | | | | |
| Set-off 15 sec. | top | | 0.41 | 0.23 | 0.58 | 0.34 | 0.10 | 0.23 |
| | wire | | | | | | | |
| Set-off 30 sec. | top | | 0.13 | 0.06 | 0.24 | 0.10 | 0.03 | 0.06 |
| | wire | | | | | | | |
| Set-off 60 sec. | top | | 0.03 | 0.02 | 0.05 | 0.02 | 0.01 | 0.01 |
| | wire | | | | | | | |
| Set-off 120 sec. | top | | 0.01 | 0.01 | 0.02 | 0.01 | | |
| | wire | | | | | | | |
| set-off 10 min. (200%) | top | | | | | | | |
| | wire | | | | | | | |

| Printing gloss | | | | | | | | |
|---|---|---|---|---|---|---|---|---|
| paper gloss Tappi 75° | top | | 69.8 | 67.3 | 76.5 | 69.6 | 62.1 | 68.7 |
| print gloss Tappi 75° | top | | 89.2 | 84.6 | 91.4 | 86.2 | 72.0 | 86.7 |
| Delta Printing gloss | top | | 19.4 | 17.3 | 14.9 | 16.6 | 9.9 | 18.0 |
| Chemical ink drying | | | | | | | | |
| Thumb test (manual) | top | h | | | | | | |
| Thumb test (manual) | wire | h | | | | | | |
| Thumb test (Fogra)* | top | h | 2 | 2 | 2 | 1 | 1 | 1 |
| Thumb test (Fogra) | wire | h | | | | | | |
| White gas test | top | h | 2-3 | 2-3 | 7 | 2-3 | 1-2 | 2-3 |
| White gas test | wire | h | | | | | | |

### Conclusions:

### Different top coatings on Standard middle coating (PC_3):

Addition of 5 and 10% silica (Syloid C803) leads to a stepwise increased short time ink setting speed (set off) which is not advantageous for runnability at printing press but set off level can be slowed down by an appropriately increased latex amount.

The higher the amount of silica used in top coating formulations the faster are the analysed white gas test values (chemical ink drying). With 10% of Syloid C803 chemical ink drying is improved from 7 hours (reference) to 1-2 hours.

The higher silica amount in top coating the lower is paper gloss level of produced paper.

General fast short time ink setting is also responsible for low print gloss values - for further improvements latex level can be increased to damp this unwanted print gloss decrease slightly.

### Experimental results, part 7

For verification a further set of experiments was carried out with the formulations for the middle coatings as given in table 2 and with top coatings according to table 14.

**Table 14 Formulations of top coatings**

| Top coat | | TC 1 | TC 3 |
|---|---|---|---|
| trial order | solid | | |
| | [%] | | |
| HC 60 | 78 | 3 | |
| HC 90 | 76.5 | 15 | |
| Pigment SFC | 72 | 72 | 77 |
| Pigment Syloid C803 | 98 | | 8 |
| Amazon | 72 | 10 | 15 |
| | | | |
| Acronal | 50 | 6.5 | 8.5 |
| Latex | 50 | 1 | 1 |
| CMC | 93.5 | 0.5 | 0.5 |
| PVOH | 20 | 1.2 | 1.2 |
| Fluocast | 50 | 0.55 | 0.55 |
| Polysalz S | 45 | 0.1 | 0.1 |

### Experimental results, part 8

A further more detailed analysis was carried out in order to assess the possibility of using chemical drying aids in the coatings in combination with silica and in order to test the possibility of using the papers according to the present invention without having to use anti-set-off powder and/or infrared drying and/or without overprint varnish. Anti Set-off Powders are blends of pure food starches with anti-caking and flow agents added and are available in a wide range of particle sizes (~ 15 to ~ 70 µm). The starch can be tapioca, wheat, maize, or potato. When sprinkled over the printed surface, it prevents the front or printed side of a substrate from intimately contacting the back or unprinted side of a substrate. The starch particles act as spacers so air can enter from the sides and between the front and back of the substrate. This free flow of air across the inked surface allows inks that "dry" or cure by surface oxidation to receive exposure to oxygen in the air. The ink then cures to its final oxidized state.
Offset powder obviously plays a very important role in a converting application that uses inks requiring oxidation to reach their final properties. Although offset powders are very beneficial, they can contribute detrimental characteristics. In applications in which a printed substrate is subject to further converting when perfect surface appearance is a requirement, use of offset powders may not be appropriate. E.g. in case of a printed substrate that will undergo lamination with an adhesive to a clear film. The application may be a label on which gloss and an optically perfect appearance are necessary. The dusting of offset powder acts like a sprinkling of dirt or other contaminant: It will produce surface imperfections in the laminate and seriously detract from the final appearance. They become entrapped in the lamination and contribute a "hills-and-valleys" appearance. This may be on a very small scale, but it is often enough to lead to an unsatisfactory appearance on close inspection. Another application in which the use of offset powder may not be appropriate is on a printed substrate used to make labels for the in-mould label process. In this process, a label printed on a paper or plastic substrate becomes an integral part of an injection- or blow-moulded container during the moulding operation. For the popular "no-label" look, the optical characteristics must be such that the consumer cannot see the label under any circumstances. Specks of offset powder, dust, or anything similar would detract from the appearance of such a label and make it unsatisfactory. Therefore the need for finding paper a substrates which eliminate the use of such powders. On a conventional woodfree paper coatings were applied with formulations as given in the subsequent tables, wherein the substrate was coated on both sides with a precoat layer in a coat weight of 11 gsm, and a top coat layer of also 11 gsm.
The formulations of the precoat layers as investigated are given in table 15, and the formulations of the top coat layers and how they are combined with the precoat layers is given in table 16:

**Table 15 Formulations of precoatings**

| pre coat: | | | V6 | V7 | V8=V6 | V9=V6 | V10=V6 | V11=V6 | V12=V7 |
|---|---|---|---|---|---|---|---|---|---|
| | | solids [%] | | | | | | | |
| HC 60 M HH | | 78 | | 43 | | | | | 43 |
| HC 90 | | 75 | | 45 | | | | | 45 |
| HC 95 M HH | | 78 | 100 | | 100 | 100 | 100 | 100 | |
| | | | | | | | | | |
| Pigment Syloid C803 | | 99.4 | | 12 | | | | | 12 |
| | | | | | | | | | |
| Binders / additives | | | | | | | | | |
| Latex | | 50 | 9 | 11.5 | 9 | 9 | 9 | 9 | 11.5 |
| PVOH | | 22 | 0.3 | 0.3 | 0.3 | 0.3 | 0.3 | 0.3 | 0.3 |
| Polysalz S | | 40 | | 0.1 | | | | | 0.1 |

**Table 16 Formulations of top coat**

| | | | IID_6 | IID_7 | IID_8 | IID_9 | IID_10 | IID_11 | IID_12 |
|---|---|---|---|---|---|---|---|---|---|
| pre coat: | | | V10 | V12 | V8 | V9 | V6 | V11 | V7 |
| top coat | | | D6 | D7 | D8 | D9 | D10 | D11 | D12=D6 |

| | | solid [%] | | | | | | | |
|---|---|---|---|---|---|---|---|---|---|
| HC 60 M HH | | 78 | 3 | 3 | | | | | 3 |
| HC 90 | | 75 | 15 | 15 | | | | | 15 |
| HC95MHH | | 78 | | | | | | | |
| SFC | | 72 | 72 | 72 | 77 | 73 | 70 | 77 | 72 |
| Amazon 88 | | 74 | 10 | 10 | 15 | 15 | 15 | 15 | 10 |
| Pigment Syloid C803 | | 99.4 | | | 8 | 12 | 15 | 8 | |
| | | | | | | | | | |
| | | | | | | | | | |
| Latex Acronal | | 50 | 8.0 | 8.0 | 10.0 | 10.0 | 10.0 | 10.0 | 8.0 |
| Latex | | 50 | 1.0 | 1.0 | 1.0 | 1.0 | 1.0 | 1.0 | 1.0 |
| PVOH | | 22 | 0.5 | 0.5 | 0.5 | 0.5 | 0.5 | 0.5 | 0.5 |
| Polysalz S | | 40 | 0.1 | 0.1 | 0.1 | 0.1 | 0.1 | 0.1 | 0.1 |
| Manganese Acetate | | 100 | 1.5 | | | | | 1.5 | 1.5 |

All coatings have good runnability without scratches and there is a high glossability of the papers - paper gloss level (55% DIN 75°) was reached with 200 kN/m nip load. The higher the silica amount used in top coating, normally the lower the paper gloss. Addition of manganese acetate has no significant influence on paper gloss. Use of silica in pre coating leads to slightly lower paper gloss of top coated paper (before calendering).

Preferentially Mn(II)acetate is used because of many advantages above other catalyst systems, and it has to be pointed out that the use of such manganese complexes is, as already pointed out above, is not limited to the present coatings but can be extended to any other coating. The manganese acetate system is characterised by no smell, a lower price, more easily water soluble salt, smaller effect on brightness/shade, no environmental/health issues. As a matter of fact for full catalytic activity of such a system, it seems to be advantageous to have Mn(II) as well as Mn(II) in the coating (top coating or second coating beneath the top coating) at the same time. Optimum activity is achieved if Mn(II) and at least some III)acetate is present. One advantageous way to intrinsically introduce necessary Mn(III)acetate next to II-form at the same time creating a minimum amount of generally brownish and in fact rather water insoluble Mn(III) form is possible as follows:
a) addition of additional 0.1pph Polysalz, in order to keep Mn-ions fully available as free catalytic species. It is suspected that if this constituent is not added, then most probably high valency Mn-ions will strongly interfere or even be bounded with calcium carbonate dispersions in coating, and will destabilise/coagulate them via interaction with double layers, so also coat quality is decreased,
b) Mn(acetate) is slowly added as last component to topcoat composition, where it is preferred to start with most pH = 8,5 - 9. Higher pH up to 10 is possible and the result (some Mn(III)) is only satisfactory but the dissolving behaviour of Mn(acetate) is then better/quicker,
c) after dissolving Mn(acetate) (as visually judged) it is also preferred to again adjust pH up to approximately 8,5 (pH generally goes down when dissolving acid reacting Mn(acetate)),
d) Finally it seems to be beneficial to have additional mixing time (typically 30 minutes in present praxis) to fully dissolve Mn(acetate) to molecular level to have it all available for catalytic cycle.
Mn(acetate) is preferably present 0,1 - 0,6% Manganese (=II+III) in weight of the total dry weight of a top coating. Most preferred is the presence of 0,2-0,4%. It has to be noted that other Mn-salts/complexes are also possible, like Mn(II)acac. The sole catalytic activity of Mn(acetate) can be enhanced and/or supported via different measures: A) combination with secondary driers and/or auxiliary driers, B) combination with responsible ligands, so e.g. combined with bpy the activity is very high and almost equal to a system like Nuodex/bpy, so combined with other ligands activity can be significantly increased to attractive level, C) addition of systems like Li(acac), D) addition of peroxides (in properly stabilized but available form) to have necessary oxygen direct at spot without diffusional limitations. As one can see from figures 28 and 29, showing the white gas test and the wet ink rub test results, respectively, paper IID_7 with reference top coating and silica in pre coating shows slowest chemical drying tendency in laboratory. With silica in top coating it is possible to reach chemical drying times of 3 or 2 hours (for higher silica amounts). Paper IID_11: use of manganese acetate in combination with 8% silica led to a further improvement 2 hours (instead of 3 hours). In this case also the dot (more critical than tail) on tested paper is dry between 3 to 4 hours. Use of silica leads to improved wet ink rub behaviour in laboratory. Addition of manganese acetate or silica in pre coating leads to further improvements.

**Table 17 Numerical set off values for IID_6 to IID_12**

| | | IID_6 | IID_7 | IID_8 | IID_9 | IID_10 | IID_11 | IID_12 |
|---|---|---|---|---|---|---|---|---|
| | | | | | | | | |
| Set Off 15 sec | Top | 0.48 | 0.68 | 0.16 | 0.02 | 0.01 | 0.25 | 0.26 |
| Set Off 30 sec | Top | 0.08 | 0.29 | 0.02 | 0.01 | 0 | 0.02 | 0.1 |
| Set off 60 sec | Top | 0.01 | 0.02 | 0 | 0 | 0 | 0 | 0 |
| Set Off 120 sec | Top | 0 | 0 | 0 | 0 | 0 | 0 | 0 |
| Set Off 15 sec | Wire | 0.5 | 0.63 | 0.12 | 0.02 | 0.01 | 0.12 | 0.31 |
| Set Off 30 sec | Wire | 0.13 | 0.11 | 0.01 | 0.01 | 0 | 0.02 | 0.07 |
| Set Off 60 sec | Wire | 0.01 | 0.02 | 0 | 0 | 0 | 0 | 0 |
| Set Off 120 sec | Wire | 0 | 0 | 0 | 0 | 0 | 0 | 0 |
| MCIS (200%) 2 min | Top | 0.03 | 0.07 | 0.03 | 0.01 | 0.01 | 0.02 | 0.05 |
| MCIS (200%) 6 min | Top | 0.01 | 0.01 | 0.01 | 0 | 0 | 0 | 0 |
| MCIS (200%) 10 min | Top | 0 | 0 | 0 | 0 | 0 | 0 | 0 |
| MCIS (200%) 2 min | Wire | 0.04 | 0.06 | 0.04 | 0.03 | 0.01 | 0.02 | 0.03 |
| MCIS (200%) 6 min | Wire | 0.01 | 0.01 | 0.01 | 0 | 0 | 0 | 0 |
| MCIS (200%) 10 min | Wire | 0 | 0 | 0 | 0 | 0 | 0 | 0 |

As one can see from figures 30 to 32, and from table 17 above, slowest ink setting is observed for paper IID_7 with silica in pre coating and reference top coating without silica or manganese acetate. An increased silica amount in top coating leads to faster initial ink setting behaviour. Use of silica in pre coating results in a slightly faster set-off compared to pre coating without silica. Short time as well as long time ink setting values are extremely small. Offset suitability (dry) as well as multi colour fibre picking level of all papers is rather low (offset suitability in most cases 0 - best valued for paper IID_7).

The specific chemical drying aid used in these experiments is Mn(II)(Ac)₂ · 4 H₂O. It should be noted that this specific transition metal complex is a highly efficient chemical drying aid, and, while it shows synergistic effect in combination with silica, it is a generally useful chemical drying aid for use in top coatings or in precoatings. One of its advantages is its price but also the stability, the ease of handling and the fact that it hardly influences the colour of the coatings provided with this chemical drying aid.

### Printing properties:

Papers tested (all 135g/m²): Scheufelen (manufacturer), BVS +8 (Name); D6; D7, D8, D9, D10; D 11; D12 (all as given above). Printing conditions: Printer: Grafi-Media (Zwalmen, N1); Press: Ryobi 5 colours; Inks in order of colour sequence: Sicpa Tempo Max B, C, M, Y; Printing speed: 11.000 sheets/h; anti-set-off powder: yes / no; Infra Red dryers: no. Tests performed: Folding: cross fold (1 buckle, 1 knife, no creasing); Wet ink rub; White gas test; Blocking test (no anti-set-off powder). Testing times: ½ hour, 1 hour, 2 hours, 3 hours, 4 hours, 24 hours, >48 hours.

### Results Blocking test:

- D6: Slight markings in 300% area
- D7: Very slight markings (better than D6)
- D8: Very slight markings in 300% area (~ D6)
- D9: No markings
- D10: No markings
- D11: Very slight markings in 300% area (a bit more than D6, but less than BVS+)
- D12: Slight markings in 300% area (a bit more than D6, but less than BVS+)
- BVS+: Markings
- D8 with powder: No markings
- D11 with powder: No markings
- BVS+ with powder: No markings
No paper presents blocking. The papers printed with anti-set-off powder do not present any markings. The paper with the most markings is BVS+. D9 and D10 (and also D8 and D11 to a slightly lesser extent) do not present any markings: they are printable without anti-set-off powder.

### Results Folding test:

The folding test has been done on a buckle folder. Contrarily to printer Haletra, there is no creasing module for the second fold, so that the folding is a bit less critical. The folding test is evaluated with help of a mark from 0 (no markings visible) to 5 (very strong markings). The results of the folding taste are summarised in table 18.

**Table 18 Results of the folding test**

| **Paper** | **½hr** | **1 hr** | **2 hr** | **3 hr** | **4 hr** | **∞** |
|---|---|---|---|---|---|---|
| D6 | 1.00 | 1.25 | 1.00 | 1.00 | 1.00 | 0.25 |
| D7 | 0.75 | 0.75 | 0.75 | 0.75 | 0.75 | 0.75 |
| D8 | 0.25 | 0.25 | 0.25 | 0.25 | 0.25 | 0.25 |
| D9 | 0.50 | 0.50 | 0.50 | 0.50 | 0.50 | 0.50 |
| D10 | 0.75 | 0.75 | 0.75 | 0.75 | 0.75 | 0.75 |
| D11 | 0.75 | 0.75 | 0.75 | 0.75 | 0.75 | 0.75 |
| D12 | 1.00 | 1.00 | 1.00 | 1.00 | 1.00 | 0.75 |
| BVS+ | 1.00 | 1.00 | 1.00 | 1.00 | 1.00 | 0.75 |
| D8 with powder | 0.25 | 0.25 | 0.25 | 0.25 | 0.25 | 0.25 |
| D11 with powder | 0.75 | 0.75 | 0.75 | 0.75 | 0.75 | 0.75 |
| BVS+ with powder | 0.25 | 0.25 | 0.25 | 0.25 | 0.25 | 0.25 |

The general level of markings at the fold has been evaluated by a group of experts (printers) as very good. There is little to no difference in the markings between ½ hour and ∞ (= a week), which would imply that the chemical drying has small effect on the folding test. There are only small differences between the papers.

### Results Wet Ink rub:

The wet ink rub test has been performed on the printed sheets, on the 300% area B, C, M. The results of this test are summarised graphically in figure 35. All papers show a very good level of wet ink rub in general. The best paper is D11, followed by D7, D8, then D9 and D10. D6, D12 and BVS+ have similar levels of markings.

### Results White gas test:

The white gas test has been performed on the printed sheets, on the 300% area B, C, M.

The results are summarised in table 19.

**Table 19 White gas test results**

| **Paper** | **White gas drying time (hr)** |
|---|---|
| D6 | 4<t<24 |
| D7 | 3 |
| D8 | ≥4 |
| D9 | 1/2 |
| D10 | 1/2 |
| D11 | 3 |
| D12 | ≥4 |
| BVS+ | 4<t<24 |
| D8 with anti set-off powder | ≥4 |
| D11 with anti set-off powder | 3 |
| BVS+ with anti set-off powder | 4<t<24 |

The fastest papers are D9 and D10, which are dry after ½ hour. The slowest paper is BVS+, followed by D6.

The following conclusions can be drawn from this experimental part:
- D9 and D10 are printable without any anti-set-off powder.
- D7, and also D11 are also printable without anti-set-off powder (only slight markings on critical areas)
- For the wet ink rub test, the levels are very good, but D11, followed by D7 and D8 showed the best results.

### Experimental results, part 9

In order to further characterise the coatings which can be used in accordance with the present invention, mercury intrusion measurements were made to determine the porosity of the final coating. Coatings which, apart from the constituents given below, are substantially identical as the ones given above were prepared as follows:
- trial_2:: 10% silica A in pre coat + 20% silica A in top coat
- trial_3:: without silica A in pre coat + 20% silica A in top coat
- trial_5:: without silica in pre coat and top coat, reference
- trial_6:: 10% silica B in pre coat + 20% silica B in top coat
wherein A is Gasil 35 M, and B is Syloid C803.

The results of the Mercury intrusion measurements are given in figure 34. In comparison with the reference one notices that in the range below 0.02 µm, i.e. in particular in the range between 0.01 and 0.02 µm, the porosity of the coatings according to the invention is higher than the one of the reference. One therefore notices an increased porosity ("peak") in and partly also below this range, which is likely to contribute and to be key to the physical ink adsorption process.

### Materials:

Inorganic pigments: The particle size distributions of used inorganic pigments are given in figure 35. The proper choice of the particle size distribution is important for the final paper and print gloss and for the ink setting properties. SFC stands for a steep fine carbonate with a specific surface area of 18 m²/g.

Silica: Chemical ink drying tendency of all silica containing papers was extremely fast - also other types of silica (Sylojet 710A and Sylojet 703A also from Grace Davison) are working (not only Syloid C803). Syloid C803 is used because this product is available as powder which allows higher solids content of coating colour and is cheaper than others. Some of the main properties of the silica are summarised in table 20.

**Table 20: Properties of silica used**

| Product | Pore Volume (ml/g) | Average particle size (µm) | Surface area (m²/g) | Surface charge | pH | Oil adsorption | Solids content (%) |
|---|---|---|---|---|---|---|---|
| Sylojet P403 (= Syloid C803) | 2.0 | 3.5 | 330 | Anionic | 3.5 | 320 | 99 |
| Sylojet 703A | 0.7 | 0.3 | 250 | Anionic | 8 | | 20 |
| Sylojet 710A | 0.9 | 1.0 | 250 | Anionic | 8 | | 20 |

Use of silica in pre coating colour in combination with standard top coating colour improves ink drying (investigated in laboratory) significantly.

Binders: all the binders mentioned here are a commercially available and therefore their properties are accessible to the public. For example Litex P 2090 is an aqueous dispersion of a copolymer of styrene and n-butylacrylate. Acronal S360D is a copolymer of styrene and acrylic ester available from BASF, DE.

### LIST OF REFERENCE NUMERALS

- 1: substrate
- 2: second layer
- 3: top layer
- 4: coated printing sheet

## Claims

1. Coated printing sheet for sheet-fed offset printing with an image receptive coating layer on a paper substrate, **characterised in that** the printing sheet can be printed in an offset printing process without spraying a fine powder on the sheet as it comes off the press to prevent the ink from transferring to the back side of the next sheet and/or without irradiative or heat drying on the sheet fed press and/or without use of overprint varnish.

2. Printing sheet according to claim 1, **characterised in that** it has a set off value of less than 0.4 measured 15 seconds after printing.

3. Printing sheet according to claim 2, **characterised in that** it has set off value of less than 0.05, preferably of less than 0.025 measured 15 seconds after printing.

4. Printing sheet according to one of the preceding claims, **characterised in that** it has a set off value of less than 0.05 measured 30 seconds after printing, preferably a set off value of less than 0.01 measured 30 seconds after printing.

5. Printing sheet according to one of the preceding claims, **characterised in that** it has a multicolour ink setting value of less than 0.04 measured two minutes after printing.

6. Printing sheet according to claim 5, **characterised in that** it has a multicolour ink setting value of less than 0.02, preferably of less than 0.015 measured two minutes after printing.

7. Printing sheet according to any of the preceding claims, **characterised in that** it has a multicolour ink setting value of less than 0.01 measured six minutes after printing, preferably of less than 0.005 measured six minutes after printing.

8. Printing sheet according to any of the preceding claims, **characterised in that** it has a set off value of less than 0.05, preferably of less than 0.02 measured 15 seconds after printing and a that it has a multicolour ink setting value of less than 0.04 measured two minutes after printing.

9. Printing sheet according to any of the preceding claims, **characterised in that** the image receptive coating layer comprises a top layer and/or at least one second layer below said top layer, said top and/or second layer comprising:
a pigment part, wherein this pigment part is comprises
a fine particulate carbonate and/or a fine particulate kaolin and/or a fine particulate silica and/or a fine particulate plastic pigment or a mixture thereof, at least one of its constituents with a surface area in the range of 18 or 40-400 m²/g, preferably of 100-400 m²/g, or in the range of 200-350 m²/g,
and a binder part, wherein this binder part is composed of:
binder and additives.

10. Printing sheet according to claim 9, **characterised in that** the pigment part comprises at least 5 parts in dry weight of a fine particulate carbonate and/or a fine particulate kaolin and/or a fine particulate silica with a particle size distribution such that the average particle size is in the range of 0.1-5 µm, preferably in the range of 0.3-4 µm.

11. Printing sheet according to any of the preceding claims, **characterised in that** the silica has a pore volume above 0.2 ml/g, preferably above 0.5 ml/g, even more preferred above 1 ml/g.

12. Printing sheet according to any of claims 9, 10 or 11, **characterised in that** at least a fraction of the inorganic pigment part, preferably fine particulate silica, comprises or is selectively enriched in traces of metals, preferably of transition metals, wherein at least one metal is present in more than 10 ppb, preferably more than 500 ppb.

13. Printing sheet according to claim 12, **characterised in that** Co, Mn, V, Ce, Fe, Cr, Ni, Rh, Ru, or combinations thereof, preferably present in the pigment in more than 10 ppb up to 10 ppm, possibly in combination with Zr, La, Nd, Al, Bi, Sr, Pb, Ba or combinations thereof, preferably present in the pigment in more than 10 ppb up to 10 ppm or 20 ppm, possibly in combination with Ca, K, Li, Zn and combinations thereof, preferably present in the pigment in more than 10 ppb up to 10 ppm or 20 ppm.

14. Printing sheet according to claim 13, **characterised in that** a combination selected from Co + Mn, Co + Ca + Zr or La or Bi or Nd, Co + Zr/Ca, Co + La, Mn + K and/or Zr.

15. Printing sheet according to any of claims 9-14, **characterised in that** the pigment part is composed of
0 - 99, preferably 80-95 parts in dry weight of a fine particulate carbonate and/or of a fine particulate kaolin
1 - 99, preferably 6 to 25 parts in dry weight of a fine particulate silica
and a binder part, wherein this binder part is composed of:
5-20 parts in dry weight of binder and
less than 4 parts in dry weight of additives.

16. Printing sheet according to any of claims 9-15, **characterised in that** the pigment part comprises 8 - 12 parts in dry weight of a fine particulate silica, preferably 8 - 10 parts in dry weight of a fine particulate silica, with a particle size distribution such that the average particle size is in the range of 0.1-5 µm, preferably in the range of 0.3-4 µm and with a surface area in the range of 200-400 m²/g.

17. Printing sheet according to any of claims 9-16, **characterised in that** the pigment part comprises 70 - 80 parts in dry weight of a fine particulate carbonate, preferably with a particle size distribution such that 50% of the particles are smaller than 1 µm, even more preferably with a particle size distribution such that 50% of the particles are smaller than 0.5 µm, and most preferably with a particle size distribution such that 50% of the particles are smaller than 0.4 µm.

18. Printing sheet according to any of claims 9-16, **characterised in that** the pigment part comprises 10 - 25 parts in dry weight of a fine particulate kaolin, preferably 13- 18 parts in dry weight of a fine particulate kaolin, wherein preferably the fine particulate kaolin with a particle size distribution such that 50% of the particles are smaller than 1µm, even more preferably with a particle size distribution such that 50% of the particles are smaller than 0.5 µm, and most preferably with a particle size distribution such that 50% of the particles are smaller than 0.3 µm.

19. Printing sheet according to any of claims 9-18, **characterised in that** the binder part comprises 7 - 12 parts in dry weight of a binder, wherein preferably the binder part comprises a binder or a mixture of binders selected from the group consisting of latex, in particular styrene-butadiene, styrene-butadiene-acrylonitrile, styrene-acrylic, in particular styrene-n-butyl acrylic copolymers, styrene-butadiene-acrylic latexes, acrylate vinylacetate copolymers, starch, polyacrylate salt, polyvinyl alcohol, soy, casein, carboxymethyl cellulose, hydroxymethyl cellulose and copolymers as well as mixtures thereof, preferably provided as an anionic colloidal dispersion in the production.

20. Printing sheet according to any of claims 9-19, **characterised in that** the binder part comprises at least one additive selected from defoamers, colorants, brighteners, dispersants, thickeners, water retention agents, preservatives, crosslinkers, lubricants and pH control agents or mixtures thereof.

21. Printing sheet according to any of claims 9-20, **characterised in that** the top coat of the image receptive layer comprises
a pigment part comprising
70-80 parts in dry weight of a fine particulate carbonate with a particle size distribution such that 50% of the particles are smaller than 0.4 µm,
10-15 parts in dry weight of a fme particulate kaoline with a particle size distribution such that 50% of the particles are smaller than 0.3 µm,
8-15 parts in dry weight of a fine particulate silica with an average particle size between 3-5 µm and a surface area of 300-400 m²/g,
and a binder part comprising
8-12 parts in dry weight of a latex binder
less than 3 parts in dry weight of further additives.

22. Printing sheet according to any of the preceding claims, **characterised in that** its coating comprises a chemical drying aid, preferably selected from a transition metal complex, a transition metal carboxylate complex, a manganese complex, a manganese (II) carboxylate complex and/or a manganese (II) acetate complex or a mixture thereof, wherein the chemical drying aid is preferably present in 0.5 to 3 parts in dry weight, preferably in 1 to 2 parts in dry weight.

23. Printing sheet according to any of the preceding claims, **characterised in that** the top coat and/or the second layer further comprises a chemical drying aid,
wherein the chemical drying aid acts as a catalytic system and is given by a transition metal complex, preferably by a manganese complex, a manganese carboxylate complex and/or a manganese acetate or acetylacetate complex, wherein for catalytic activity of Mn complexes preferably Mn(II) as well as Mn(III) are present concomitantly, or a mixture thereof, wherein the metal part of the catalyst system is present in the coating in 0.05 - 0.6 weight-%, preferably in 0.02 - 0.4 weight-%, of the total dry weight of the coating.

24. Printing sheet according to any of the preceding claims, **characterised in that** it is calendered and/or that it is a matt, glossy or a satin paper, wherein in case of a glossy paper it is **characterized by** a gloss on the surface of the image receptive coating of more than 75 % according to TAPPI 75deg or of more than 50 according to DIN 75deg, or **characterised in** case of a matt paper by a gloss on the surface of the image receptive coating of less than 25 % according to TAPPI 75deg, or **characterised in** case of a satin paper by a gloss on the surface of the image receptive coating in the intermediate range.

25. Printing sheet according to any of the preceding claims, **characterised in that** an image receptive coating layer is provided on both sides of the substrate.

26. Printing sheet according to any of the preceding claims, **characterised in that** the substrate is a woodfree paper substrate.

27. Printing sheet according to any of the preceding claims, **characterised in that** the image receptive coating layer has a second layer beneath said top layer comprising:
a pigment part, wherein this pigment part is composed of 80- 98 parts in dry weight of a mixture of or a single fine particulate carbonate, preferably with a particle size distribution such that 50% of the particles are smaller than 2 µm,
2-25 parts in dry weight of a fine particulate silica
and a binder part, wherein this binder is composed of:
less than 20 parts in dry weight of binder, preferably 8-15 parts in dry weight of latex or starch binder,
less than 4 parts in dry weight of additives
wherein preferably the fine particulate carbonate of the pigment part consists of a mixture of one fine particulate carbonate with a particle distribution such that 50% of the particles are smaller than 2 µm, and of another fine particulate carbonate with a particle distribution such that 50% of the particles are smaller than 1 µm, wherein preferentially those two constituents are present in approximately equal amounts and/or wherein the pigment part comprises 5-15 parts in dry weight of silica, preferably in a quality as defined in claim 11 and/or 14.

28. Printing sheet according to any of the preceding claims, **characterised in that** it comprises only two coatings on the raw paper substrate.

29. Printing sheet according to any of the preceding claims, **characterised in that** it is re-printable and convertable within less than one hour, preferably within less than 0.5 hours.

30. Method for making a printing sheet according to any of the preceding claims, **characterised in that** a top coating formulation comprising a fine particulate carbonate and/or a fine particulate kaolin and/or a fine particulate silica and/or a fine particulate plastic pigment or a mixture thereof, at least one of its constituents with a surface area in the range of 18 - 400 m²/g, 40 - 400 m²/g or 100-400 m²/g, preferably in the range of 200-350 m²/g, is applied onto a precoated or on coated paper substrate, preferably on woodfree basis, using a curtain coater, a blade coater, a roll coater, a spray coater, an air knife, cast coating and/or a metering size press.

31. Method for making a printing sheet according to claim 30, **characterised in that** the coated paper is calendered at a speed of in the range of 200-2000 m/min, at a nip load of in the range of 50-500 N/mm and at a temperature above room temperature, preferably above 60° Celsius, even more preferably in the range of 70 - 95° Celsius using between 1 and 15 nips.

32. Use of a printing sheet according to any of the claims 1-29 in a sheet fed offset printing process, wherein in that offset printing process no or substantially no fine powder is sprayed on the sheet as it comes off the press to prevent the ink from transferring to the back side of the next sheet and/or no irradiative or heat drying on the sheet fed press is carried out and/or no use of overprint varnish is made.

33. Use of a printing sheet according to claim 32 wherein in that process reprinting and converting takes place within less than one hour, preferably within less than 0.5 hours.
